

Patented Aug. 16, 1949

2,479,311

# UNITED STATES PATENT OFFICE

2,479,311

## PRODUCTION OF OXYGEN-FREE COPPER

Arthur L. Christensen, Perth Amboy, N. J., and  
Horace F. Silliman, Waterbury, Conn., assign-  
ors to International Smelting and Refining  
Company, a corporation of Montana

No Drawing. Application July 11, 1945,  
Serial No. 604,500

2 Claims. (Cl. 75—76)

1

This invention relates to the production of oxygen-free copper and has for its object the provision of an improved method of producing substantially oxygen-free copper of high electrical conductivity.

The present invention is a variant of the invention disclosed in the copending application of Christensen, McKean and Silliman Ser. No. 560,898, filed October 28, 1944, now abandoned, wherein boron is used to degas copper rather than to deoxidize it. As pointed out in that application, it is extremely difficult to melt copper without picking up some oxygen. This is true even in an induction furnace, because of the exposure to the atmosphere of projecting hot ends of the copper before it is melted down. In the process of the aforementioned application, oxygen in the molten copper is removed by treating the copper with a reducing gas such as hydrogen which dissolves in the copper and removes any dissolved oxygen, and the residual dissolved hydrogen is then removed by treatment with boron. In accordance with the present invention, copper is melted down in contact with carbon or graphite heated to a temperature above the melting temperature of copper and the exposed surface of the molten copper is protected with a cover of finely divided carbon or graphite. The molten copper is effectively deoxidized by the action thereon of the hot carbon or graphite. The resulting deoxidized molten copper (preferably at a temperature of about 2200° F.) is then treated with boron to remove any dissolved reducing gases.

Electrolytically refined copper contains small amounts of arsenic, antimony, iron and nickel, the percentages ranging from 0.0005% up to 0.002% with arsenic and antimony present in the lesser amounts. When making tough pitch wire bars this copper has an electrical conductivity ranging from 100.5% to 101.5% I. A. C. S. It contains 0.02% to 0.05% oxygen, largely present as cuprous oxide on the grain boundaries, but this oxygen has placed some of the impurities such as arsenic, antimony, iron or nickel on the grain boundaries as well. Tough pitch copper with this conductivity can be treated with carbon to remove all the oxygen, cast and drawn into oxygen-free copper wire which will have a conductivity ranging from 100.0 to 101.0%. The removal of oxygen has placed the impurities in solution in the copper with the result of a 0.5% drop in conductivity. The A. S. T. M. specifications for high conductivity copper include the requirement of a 100.0% conductivity. Generally the refiner sets his own requirement at 100.5% allowing himself a 0.5% factor of safety because of minute errors and variations that can develop in the preparation and testing of the wire. It is therefore evident from the foregoing figures that when degassing or deoxidizing copper any form of contamination

2

must be avoided and the residual excess of the degassing or deoxidizing element must be very carefully controlled. Although boron has less effect on reducing the conductivity of copper than most other elements, it has nevertheless sufficient effect so that it must be maintained in the copper at less than 0.02%, if the A. S. T. M. specification for conductivity is to be met.

Smooth deposition of copper in an electrolytic refinery is obtained by including in the copper electrolyte certain colloidal addition agents which, to some extent, become imbedded in the deposited cathode copper. Animal glue, a wood pulp mill residue known as goulac, and some so-called water soluble mineral oils are examples of such addition agents. High quality copper cathodes show an ignition loss of 0.015% of which only 0.0015% is sulphur. The remainder is largely organic matter that breaks down in molten copper to various other compounds of carbon, hydrogen, oxygen and nitrogen with residual hydrogen, hydrogen sulphide and probably other reducing gaseous impurities remaining in the molten copper. The heretofore generally accepted practice of producing sound oxygen-free copper is to expose the molten cathode copper to air with the result that a certain oxygen pick-up in the copper effects a removal of these reducing gaseous impurities. The oxygen is then removed with calcined charcoal, carbon monoxide free of water vapor and hydrogen, or by the use of some deoxidizing element such as phosphorus, lithium, boron, etc. Any substantial residual excess of the deoxidizing element lowers the electrical conductivity of the copper, and hence it is difficult to economically produce high conductivity oxygen-free copper by these practices. Contrasted with this heretofore generally accepted practice, the present invention first deoxidizes the molten copper by contact with hot carbon or graphite and retains in the deoxidized molten copper the reducing gases resulting from the decomposition of occluded addition agents, electrolyte and moisture. The reducing gases are then removed by the boron treatment, which requires less boron than is required when boron is used as a deoxidizing element. Moreover, the invention provides more precise control over the residual boron content of the copper.

Some metals have the property of picking up carbon, and where carbon pick-up has to be avoided it is not possible to take advantage of the rapid induction furnace heating rate to be obtaining when using a graphite crucible. It has been found that copper also picks up carbon, but only in very small amounts and under special conditions. Consequently, for all practical purposes copper is not contaminated by melting in graphite or carbon. The present invention takes

advantage of this circumstance, and contemplates melting copper in a carbon or graphite crucible or the like heated to a temperature above the melting temperature of copper and protecting the exposed surface of the resulting molten copper by a cover of finely divided or pulverized carbon or graphite. Since the carbon or graphite crucible is hotter than the molten copper, any oxygen in the copper is effectively removed, and the copper is thereby deoxidized, by contact with the hot carbon or graphite. This deoxidation is so effective and complete that no special treatment of the copper with reducing gases is necessary prior to the boron treatment. As soon as all the copper is molten the surface of the molten copper is covered with powdered carbon or graphite so as to avoid contact with the air, and there is then no possibility for reoxidation of the copper. At this stage, the molten copper is oxygen-free, but it contains dissolved reducing gases. In accordance with the present invention, these reducing gases are then removed from the molten copper by treatment with a boron-containing agent, preferably a boron-copper alloy, in amount insufficient to introduce into the treated copper such an amount of residual boron as to objectionably reduce its electrical conductivity.

The reducing gases in the deoxidized molten copper originate for the most part from impurities in the copper. Cathode copper is a particularly desirable form of copper for the production of oxygen-free high conductivity copper, and customarily contains traces of organic matter and traces of occluded electrolyte and moisture. In the course of the melt down and deoxidation of the copper by contact with hot carbon or graphite, the impurities are largely converted to reducing gases such as hydrogen, hydrogen sulphide and probably some hydrocarbons which may not crack at the prevailing temperature. These reducing gases are dissolved in the oxygen-free molten copper and are effectively removed by the boron treatment. Since the copper contains no oxygen, the boron is not a deoxidizing agent, and only a relatively small amount is required to remove the dissolved reducing gases. From 0.005 to 0.02% of boron based on the weight of the molten copper treated is sufficient for the purpose, and ordinarily about 0.01% boron by weight gives entirely satisfactory results. The boron is preferably introduced into the molten copper in the form of a master alloy of boron and copper containing from 0.5 to 5% boron and the balance copper with less than 1% impurities. Such a boron-copper alloy admirably adapted for the practice of the invention is made in accordance with Silliman Patent No. 2,195,433, and contains 3 to 5% boron, around 95% copper and less than 1% impurities (mostly iron, silicon and magnesium).

In practicing the invention, the copper is preferably melted in a graphite crucible of a coreless induction furnace. With a graphite crucible, the furnace operates under a very steady power load because the crucible absorbs all the eddy currents. The crucible becomes the hottest part of the furnace and the copper is melted entirely by conduction of heat from the crucible. Graphite is the preferred form of carbon because it is more dense and burns away less rapidly than other available forms of carbon. The graphite or other form of carbon should be of high purity such for example as high quality Acheson graphite. Although induction heating is preferred, the graphite or carbon crucible may be locally heated

in any appropriate manner, as for example by electric resistance heating units.

The crucible or the like may be made of or lined with carbon or graphite in various ways. In a small coreless induction furnace, the crucible may be lined with a plastic graphite mix containing a carbonaceous binder, such, for example, as pitch or sugar solution. In larger furnaces, pre-formed circle block linings may be used, with graphite paste bonded joints. It is our present preferred practice to turn out the crucible from high quality Acheson graphite electrodes. Such electrodes are now available with diameters up to 24 inches. A suitable crucible wall thickness is 3 inches and it is thus possible to develop inside dimensions of 18 inches in diameter by about 30 inches high which is a shape that allows a satisfactory furnace design. Such a crucible can produce about 2000 pounds of oxygen-free high conductivity copper per heat in a period of 60 to 90 minutes.

In addition to its action in deoxidizing the molten copper, the carbon or graphite crucible is of special advantage with respect to the boron treatment of the molten copper. Boron is an extremely energetic reducing agent, and reacts with the metal oxides and silicates commonly present in many furnace refractories, thereby forming free metals (e. g. silicon and iron) which very deleteriously affect the electrical conductivity of the copper. For example, small amounts of silicon and iron, say 0.005% of each, have a very noticeable detrimental effect on the conductivity of copper. Carbon and graphite are not only resistant to this action of boron, but are available in such pure state as not to contaminate the boron-treated copper.

The following example illustrates an actual practice of the invention in a 125 kw. coreless induction furnace having a crucible turned out of a highest quality Acheson graphite electrode. The boron treatment was carried out with a boron-copper alloy containing 3% boron, 0.6% impurities consisting mainly of magnesium, silicon and iron, and the remainder copper. The steps in the process were as follows:

(1) After casting out the previous charge of boron-treated copper, the crucible was immediately filled with cut copper cathodes of a size which stacked in the crucible sufficiently well so as to require only about two additional rechargings in order to finally develop a full crucible of molten copper. Prior to the start of recharging and during this entire melting period the full load of the motor generator was on the furnace coil. In this case the watt meter on the output side of the generator showed 100 to 115 kw. The load was practically constant throughout the entire period because the crucible was drawing all the power and as a result of this condition it was not necessary to make the power adjustments normally required when using a less conductive crucible. During this melt-down period pulverized Acheson graphite varying in size from 20 mesh to minus 200 mesh was added so as to cover the bath of copper. When the crucible was partly full of molten copper the charged cathodes would submerge and there was bubbling from traces of organic matter and traces of occluded electrolyte and moisture previously mentioned.

(2) In 50 minutes time the copper was entirely molten and as the last piece melted the power was immediately shut off. The crucible was still much hotter than the copper but in a few minutes time the temperature was uniform. More pul-

verized graphite was placed on any exposed surface of the bath. The temperature was then taken with an optical pyrometer sighting into a closed end target tube submerged in the bath. If the temperature was 2200° F. treatment with the master alloy was made. If less than 2200° F. some additional heating was done.

(3) During this period the copper molds had been stripped from the previous castings, cooled to about 200° F. with water, then placed in their normal vertical position on rails and spray-coated with a water dispersion of finely ground Dixon graphite and lampblack in a ratio of about 8-5-1-0.2 water-graphite-lampblack-tannic acid by weight. With a few minutes of standing with bottoms open on rails the molds were dry and they were then placed on the cast iron base plates in line to receive the treated copper. The base plates were not dressed. Cleaner, smoother surfaces were obtained by not dressing the base plates.

(4) The copper in the furnace crucible was treated with the required boron by wiring paper bags containing the boron-copper alloy (3% boron) to graphite rods, submerging under the powdered graphite cover and stirring until dissolved. This stirring required 10 to 15 seconds.

(5) In order to prevent air from sweeping into the crucible, while tipping to cast, a clay-graphite crucible cover was placed on the crucible. This cover was 4 to 6 inches away from the molten copper but it prevented a sweep of air into the crucible, confined and maintained a carbon monoxide atmosphere over the bath as a result of the burning powdered graphite. This cover minimized boron losses during casting.

(6) The crucible was tipped until just ready to pour and then the powdered graphite was pushed back from the lip sufficiently to get a clean pour started. Thereafter the graphite did not travel out of the crucible with the copper but remained back toward the bottom of the crucible and it was possible to empty the copper completely without a detrimental amount of graphite carrying out into the mold. This inert and slightly cohesive character of Acheson graphite powder makes it an ideal cover for molten copper. Charcoal and other carbonaceous materials generally require calcination prior to use in this way in order to avoid gassing the copper. Dry Acheson graphite requires no treatment prior to use. It is also maintained on the bath in a more easily controlled manner and does not require a bottom pour ladle or any other special means to prevent carrying over into the molds.

(7) When the one mold had been filled with copper it was necessary to wait until freezing had started and refill once or twice, depending on the size of the casting, so as to make up for the shrinkage which occurs when copper passes from the molten to the solid state. This casting and filling of the shrink hole required 3 to 5 minutes for each casting. The empty furnace was then tipped back to melting position, the clay-graphite cover was removed and recharging of cathodes was started with the power on the furnace again.

The copper produced in the foregoing example was oxygen-free, possessed high electrical conductivity, superior working properties, and the high density characteristic of high quality boron-treated copper. The boron-copper alloy was used in three different amounts so as to treat the copper with 0.01%, 0.015% and 0.02% by weight of boron. The degree of control obtained by the induction furnace heating was so precise that the

electrical conductivities of castings resulting from an 0.02% boron treatment were 0.65% lower than castings resulting from an 0.01% boron treatment. The average results of nine castings from each of the three boron treatments were as follows:

| Per cent Boron Added                                  | 0.01   | 0.015        | 0.02   |
|-------------------------------------------------------|--------|--------------|--------|
| Average Per Cent Conductivities                       | 100.67 | 100.25       | 100.02 |
| Average 90° Bends after 30 min. H <sup>2</sup> anneal | 13.6   | 14.2         | 15.0   |
| Average Densities                                     | 8.88   | 8.89 to 8.91 |        |

The foregoing results indicate a precision of control not obtainable with any of the heretofore generally accepted practices for producing oxygen-free high conductivity copper. Oxygen-free copper with a residual boron content of 0.001 to 0.01% (and usually about 0.005%) can be consistently and economically produced by the invention.

We claim:

1. The method of producing substantially oxygen-free copper which comprises melting copper in contact with carbon heated to a temperature above the melting temperature of copper and protecting the exposed surface of the resulting molten copper with a cover of finely divided carbon for a sufficient period of time for the molten copper to become substantially completely deoxidized by contact with the hot carbon and to absorb reducing gases, and then removing the reducing gases from the resulting substantially completely deoxidized molten copper by treatment thereof with a boron-containing agent of the group consisting of boron and boron-copper.

2. The method of producing substantially oxygen-free copper which comprises melting copper in a carbon crucible heated to a temperature above the melting temperature of copper and protecting the exposed surface of the resulting molten copper with a cover of finely divided carbon and substantially completely deoxidizing the molten copper by the action thereon of the hot carbon of the crucible and with the absorption therein of reducing gases, and then removing the reducing gases from the resulting substantially completely deoxidized molten copper by treatment thereof with a boron-containing agent of the group consisting of boron and boron-copper in such amount as to introduce into the treated copper less than 0.02% of residual boron.

ARTHUR L. CHRISTENSEN.

HORACE F. SILLIMAN.

#### REFERENCES CITED

The following references are of record in the file of this patent:

#### UNITED STATES PATENTS

| Number    | Name            | Date          |
|-----------|-----------------|---------------|
| 1,023,604 | Weintraub       | Apr. 16, 1912 |
| 1,578,044 | Lapsley         | Mar. 23, 1926 |
| 1,955,726 | Archer et al.   | Apr. 24, 1934 |
| 2,003,889 | Jennison et al. | June 4, 1935  |
| 2,195,433 | Silliman        | Apr. 2, 1940  |

#### FOREIGN PATENTS

| Number  | Country       | Date         |
|---------|---------------|--------------|
| 423,697 | Great Britain | Feb. 6, 1935 |

#### OTHER REFERENCES

Transactions, A. I. M. M. E., vol. 104, pages 152 to 165 (1935).

1001 Alloy Formulas, by Jarvis 1927, pages 25